

T. Shaw.

Refining Iron & Steel.

No. 92,480.

Patented Jul. 13, 1869.



Witnesses;

Robert Norton

Robert Hartshorne

Inventor;  
Thomas Shaw

# United States Patent Office.

THOMAS SHAW, OF PHILADELPHIA, PENNSYLVANIA.

*Letters Patent No. 92,480, dated July 13, 1869; antedated April 30, 1869*

## IMPROVED APPARATUS FOR SHOTTING METALS.

The Schedule referred to in these Letters Patent and making part of the same.

*To all whom it may concern:*

Be it known that I, THOMAS SHAW, of the city and county of Philadelphia, Pennsylvania, have invented a new and improved Method of Shotting and Oxidizing Metals; and I do hereby declare the following to be a full, clear, and exact description of the same, reference being had to the accompanying drawing, and to the letters of reference marked thereon.

My invention consists in the forcing of molten metals in a spray, of fountain-like character, upward, in the manner and for the purpose as hereafter described.

The object of the invention is to shot and oxidize metals, without the use of towers or elevated positions.

In order to enable others to use and practise my invention, I will proceed to describe its construction and mode of operation.

On reference to the accompanying drawing, which forms part of this specification, the sketch represents a longitudinal vertical section, through the centre of appliance, adapted to creating said spray or fountain, of which *a* is a pillar supporting a curved tube or reservoir, *b*, of which *d* is the inlet and *f* the outlet.

*c* is a tube for conveying steam or other gaseous fluids, and is secured to tube *b* by soldering with block *e*, all for the purpose as hereafter described.

The object of curved tube *b* is to guide the molten metal (poured in at *d*) on a line immediately in front of a powerful blast of steam or air blowing upon it from pipe *c*, the effect of which is to blow the molten

metal in a spray violently from the mouth *f*, after which it is allowed to fall in water in the usual manner.

Both the inlet-mouth *d* and outlet-mouth *f* can be more or less closed, or the mouth *f* variously shaped, according to kind of metal operating on any kind of spray desired.

The apparatus is put in operation in this wise:

A current of air or steam is blown into tube *b* from pipe *c*, when molten metal is poured in tube *b*, in front of said blast of steam or air, the force of which throws it violently out of mouth of said tube *b* in a spray, which is allowed to fall in water. The metals will be variously oxidized, in proportion to distance thrown from mouth *f*.

It will be evident that the mouth of tube *b* can be variously shaped and closed, and that said tube or reservoir can be constructed of various materials, and modified in shape without any material alteration in result.

I do not, therefore, wish to confine myself to exact shape of apparatus; but

What I do claim, and desire to secure by Letters Patent, is—

The blowing of molten metals in a fountain into the air, whereby they are shotted, in the manner and for the purpose substantially as set forth.

THOMAS SHAW. [L. S.]

Witnesses:

ROBERT HUTCHINSON,  
ROB. POST.